

Patented Feb. 20, 1923.

1,445,645

# UNITED STATES PATENT OFFICE.

JAMES HENRY REID, OF READSBORO, VERMONT, ASSIGNOR TO THOMAS Q. HOGAN, OF BOSTON, MASSACHUSETTS.

## PROCESS OF AND MATERIAL FOR THE PRODUCTION OF METAL HYDRATES AND FOR THE PRODUCTION OF GAS.

No Drawing.

Application filed January 27, 1921. Serial No. 440,343.

To all whom it may concern:

Be it known that I, JAMES HENRY REID, a citizen of the United States, residing at Readsboro, in the county of Bennington and State of Vermont, have invented a certain new and useful Improvement in Processes of and Materials for the Production of Metal Hydrates and for the Production of Gas, of which the following is a full, clear, 10 and exact description.

This invention relates to the preparation or production of sodium or potassium hydroxide, and has for its general object to provide a process by which the said hydroxide may be secured, together with carbide material suitable for the generation of acetylene or the preparation of nitrified material; furthermore, in the practice of my process, to obtain a large quantity of gas of 20 a heating value useful in the industrial arts.

In practicing my invention, I make a mixture of cokable carbonaceous material (preferably bituminous coal) with either sodium or potassium feldspar in about the proportions of 100 lbs. of the feldspar to 41 lbs. of the coal, the feldspar and the coal having been previously reduced to a finely divided condition and intimately mingled. This mixture is then introduced into one or 30 more retorts, such as are used in the manufacture of gas or in by-product coke ovens, and is there subjected to a temperature of from 1400° F. to 2800° F. for the purpose of converting the coal into coke and securing a strong coke-like aggregate of the feldspar and coke capable of most efficient reduction in an electric furnace.

In this retorting operation, the gases which are obtainable by the ordinary distillation of bituminous coal will be evolved and, in addition, a quantity of gas produced by the decomposition of the tarry and oily constituents of the coal, this decomposition and cracking into gas of the tarry and oily products being secured through the contact of such products with the finely-divided glowing particles of the feldspar.

The only change that has been accomplished by the retorting operation is the conversion of the coal into coke, with the production of the gases above mentioned, and the production of a strong coked mixture of the feldspar with the coked coal.

This mixture, by reason of its strength and its uniformity of composition, is in ideal condition for treatment in an electric furnace, constituting an ideal uniform resistor to the passage of the electric current therethrough. The material may be supplied to any standard type of electric furnace, but I prefer a furnace of the continuous delivery type, such, for instance, as shown in my application No. 358,456 filed February 13, 1920.

In this furnace, the material will be reduced to aluminum carbide, aluminum oxy-carbide, or to a material of the nature of silicon carbide, but harder than the latter dependent upon the temperature and other conditions within the furnace.

During the carbide reaction,  $\text{Na}_2\text{O}$  or  $\text{K}_2\text{O}$  will be evolved depending, upon the use of sodium or potassium feldspar, together with a gas consisting mainly of carbon monoxide. These gases will be conducted through the hydraulic main, scrubber and other appliances generally employed in gas plants. In the scrubber, the  $\text{Na}_2\text{O}$  or  $\text{K}_2\text{O}$  will be sublimated or precipitated, forming with the water  $\text{NaOH}$  or  $\text{KOH}$ , while the carbon monoxide and other gases pass on to the holder.

With the proportion of feldspar and coal as given, the most probable solid products in the electrical furnace will be  $\text{Al}_4\text{C}_3\text{SiO}_2$ ; but, by increasing the proportion of carbon, the oxygen of the  $\text{SiO}_2$  may be taken up, leaving aluminum silicon carbide—of the nature of carborundum, but probably harder.

Having thus described my invention, what I claim is:

1. The herein described process which comprises heating in a retort sealed against the admission of air thereto a mixture of an aluminum-silicon compound of a metal with cokable carbonaceous material, reducing the solid educt from the retort in an electric furnace, thereby producing an oxide of the metal, and separating such oxide from the gases evolved during the reducing operation.

2. The process of recovering sodium or potassium and producing gas which comprises retorting a mixture of an aluminum-silicon compound of such metal with cokable carbonaceous material, collecting the evolved

gases, reducing the solid educt from the retort in an electric furnace, thereby producing an oxide of the metal, and separating such oxide from the gases evolved during the reducing operation.

3. The herein described process which comprises heating in a retort sealed against the admission of air thereto a mixture of an aluminum feldspar of a metal with cokable carbonaceous material, reducing the solid educt from the retort in an electric furnace, thereby producing an oxide of the metal, and separating such oxide from the gases evolved during the reducing operation.

15 4. The process of recovering sodium or potassium and producing gas which comprises retorting a mixture of an aluminum feldspar of such metal with cokable carbonaceous material, collecting the evolved gases, reducing the solid educt from the retort in an electric furnace, thereby producing an oxide of the metal, and separating such oxide from the other gases evolved during the reducing operation.

20 5. The herein described process comprising retorting a mixture of cokable carbonaceous material with a metal aluminum silicate, collecting the evolved gases, reducing the solid educt from the retort in an electric furnace and thereby producing gases and the oxide of such metal, collecting the evolved gases, and sublimating the said metal oxide contained therein.

35 6. The herein described process comprising heating in a retort sealed against the admission of air thereto a mixture of cokable carbonaceous material with a metal aluminum silicate, reducing the solid educt from the retort in an electric furnace and thereby producing gases and the oxide of such metal, and sublimating the said metal oxide contained in such gases.

40 7. The process which comprises retorting a mixture of cokable carbonaceous material

with an aluminum silicate of a metal, recovering the evolved gases, heating the coked mixture from the retort, with the evolution of carbon monoxide and the oxide of said metal, collecting the said gas and oxide, and separating the metal oxide from the said gas.

45 8. The process which comprises retorting a mixture of cokable carbonaceous material with the aluminum silicate of a metal, thereby to produce a coked mass, collecting the gases evolved in the retorting operation, subjecting the coked mixture to the action of electricity thereby to produce an oxide of such metal, a carbide, and a gas consisting principally of carbon monoxide, collecting such gas, and separating the metal oxide therefrom.

50 9. The process which comprises subjecting a coked mixture of cokable carbonaceous material with a metal aluminum silicate to a temperature sufficient to convert the mixture into a metal carbide, a gas containing carbon monoxide, and the oxide of such metal.

55 10. The process which comprises subjecting to electricity a coked mixture of cokable carbonaceous material with the aluminum silicate of the metal, thereby producing an oxide of such metal and a carbide, and removing the oxide by sublimation.

60 11. The process which comprises subjecting a coked mixture of cokable carbonaceous material with a metal aluminum silicate to the action of heat, thereby to produce a gas and the oxide of such metal, and separating the oxide from such gas.

65 12. The process which comprises heating a coked mixture of cokable carbonaceous material with the aluminum silicate of a metal, thereby to produce a gas and the oxide of such metal, and sublimating such oxide.

70 In testimony whereof, I hereunto affix my signature.

JAMES HENRY REID.